

FIP8309      XR      1,199,745  
 TREATMENT & CHEMICAL MODIFI-  
 CATION OF TEXTILES & FIBERS,

# 111 UNITED STATES PATENT OFFICE.

IRWIN J. SMITH, OF MENANDS, AND HARRY B. SMITH, OF ALBANY, NEW YORK,  
 ASSIGNORS TO SURPASS CHEMICAL CO., INC., A CORPORATION OF NEW YORK.

## PROCESS OF DYEING.

1,199,745.

Specification of Letters Patent. Patented Sept. 26, 1916.

No Drawing. Continuation of application Serial No. 848,152, filed June 30, 1914. This application filed March 21, 1916. Serial No. 85,548.

To all whom it may concern:

Be it known that we, IRWIN J. SMITH and HARRY B. SMITH, both citizens of the United States, and residents of Menands and Albany, respectively, in the county of Albany, State of New York, have invented a certain new and useful Process of Dyeing, of which the following is a specification.

Our invention relates to a process of dyeing cotton material.

One of the objects of our invention is to shorten the time for dyeing as well as to simplify the dyeing process and the equipment for carrying out the process as compared with prior processes and equipment therefor.

This application is a continuation of our application Ser. No. 848,152, filed June 30, 1914.

20 The kind of material to which this process is primarily adapted is unbleached knitted cotton goods containing motes, shives and, or, leaf. It is obvious that the process is applicable to any class of cotton goods or 25 yarns from which it is desired to remove the motes, shives and, or, leaf and dye the material.

In processes as heretofore used for dyeing knit or woven cotton material, it has been 30 the practice to first bleach the material and then subsequently dye it. The bleaching process was also effective to destroy specks of foreign matter, such specks consisting of motes, shives and, or leaf. A chlorin bleaching 35 process has been most generally employed. In carrying on that process the material is first boiled in an alkaline solution for a considerable time. It is then washed out and thereafter submitted to the action 40 of a solution of hypochlorites which must not be hot or it will seriously injure the material. The material is again washed out and then subjected to an acid bath to neutralize the chlorin. It is again washed out 45 and then submitted to a heated dye bath, the several operations requiring from 12 to 24 hours. A peroxid of hydrogen process also has been used to some extent and it consists in the two steps of bleaching and dyeing 50 separately, with an intermediate washing out step, and has required about 8 to 10 hours. In our process there is no separate step of bleaching, as has been heretofore considered necessary. We have discovered 55 that to dye this character of goods it is not

necessary to carry out a distinct bleaching operation as a preliminary to the dyeing of the fabric and that a satisfactory and much more economical dyeing can be effected by removing the motes, shives and, or, leafs by 60 an oxidizing bath, which is markedly alkaline, to which bath the dye is added while the material is still in the solution. To the extent that this bath has a tendency to bleach, such tendency is only incidental, the 65 whole process being carried out solely from the standpoint of removing the motes, shives and, or leaf without injury to the material and dyeing the same, and the reagents and their strength are chosen accordingly. 70

The alkaline oxidizing agent for the bath is preferably composed of about half each of peroxid of sodium and an alkaline sodium salt such as soda ash, silicate of soda, caustic soda, phosphate of soda, alone, or a mixture of any of these salts, and is used in the proportion of about 3% of the weight of the goods under treatment. Such a solution as this is strongly alkaline and at the same oxidizing and, because it is strongly alkaline, 75 the time required for removing the motes, shives, and, or leaf is much reduced as compared with any previous process of which we have knowledge. At the same time the alkalinity is not sufficiently intense to harden 80 the material to be dyed. This solution has been found to operate with entire satisfaction, but it is understood that any oxygen-liberating product, but preferably those corresponding to the "per" salts, along with 85 the above alkaline salts or certain other alkalines will give satisfactory results. For instance, peroxid of hydrogen, percarbonate of sodium, perborate of sodium, persulfate of sodium or persilicate of sodium may be 90 used with a suitable alkaline salt or mixture of salts, such as those above mentioned, although we have obtained the best results with peroxid of sodium.

Ordinarily in this class of work the material is dyed of a color and shade to imitate the natural color and shade of Egyptian cotton, goods so dyed being known in the trade as having a mock Egyptian shade. The dyes must have qualities which are substantially operatively unaffected by the oxygen-yielding compounds and alkalis. We consider that a direct or substantive dye having such a characteristic is preferable. We have, for example, employed in prac- 110

8. BLEACHING & DYEING; FLUID TREATMENT & CHEMICAL MODIFICATION OF TEXTILES & FIBERS, Cross Reference

Search Room

111

2

1,198,745

tice as a suitable dye for the purpose a mixture composed of a suitable proportion of three well known dyes having the trade names "naphthamin orange T G", "naphthamin brown R B" and "direct black G." The exact chemical compositions of these dyes are not set forth in the literature of the art, but the first two are of the naphthamin group which are diazo dyes for cotton prepared from amidonaphtholidisulfonic acid G and metanaphthylenediaminsulfonic acids. The direct black G is a substantive diazo dye stuff for cotton. We have also used satisfactorily some of the vegetable dyes as fus-  
tic, quebracho and natural tannin extracts along with direct dyes, but not with as good results as with the direct or substantive dyes alone. Our experience has been that most of the general classes of dyes to which we have referred can be satisfactorily used in our process.

We have found it preferable in our own practice of the invention to pursue a detailed procedure substantially as follows, but we do not limit our invention to this exact mode of procedure as it may be varied without departing from the invention as set forth in the appended claims: The goods are entered into a bath containing water of any convenient temperature, without a previous wetting out. The ingredients above given are then added and the bath brought to a boil. The steam is turned off and the bath allowed to cool down to about 110° F. The necessary dye stuff is then added to produce the shade desired, steam is again turned on and the bath gradually brought to a boil. It is boiled for from 15 to 30 minutes, when the steam is turned off and the bath allowed to cool down to about 190° F. and is held substantially at this temperature until the process is completed, which is about three and one-half hours from the time the agent was added. During the entire treatment the material to be dyed and the bath are given a relative movement with respect to each other so that the removal of the motes, shives and, or, leaf is uniformly and more rapidly effected and so that an even application of the dye-stuff will be made upon the material. It is immaterial how this relative movement is secured, but some relative movement is preferable in order that a uniform application may be secured. The bath is then drawn off and the goods are rinsed and whizzed.

From the above it will be seen that the time required to complete this process is only three and one-half hours. The goods are found also to be much stronger than when subjected to the chlorin process, and the shrinkage in weight is about 50% less than in that process. The labor, steam and water costs are also much reduced as compared with prior processes.

While we do not propose to be limited to any theory of the chemical reactions, we offer the following as an explanation of what probably takes place: When the material is subjected to the bath containing the alkaline-oxidizing agent, the motes, shives and, or, leaf are subjected to a chemical action which probably softens them and at the same time the material is thoroughly saturated with the alkaline solution. Before the above chemical action is complete the dye stuff is added and the material dyed during the remaining time necessary for the completion of this chemical action.

In our process a part of the time heretofore necessary for a bleaching step is utilized for simultaneously cleansing the material of motes, shives and, or, leaf and dyeing it, and by using such a strongly alkaline bath as we have described the cleansing of the material is further hastened. When the cleansing process is completed, the material has been thoroughly and uniformly dyed, thus shortening the whole process by several hours and reducing the number of operations.

During the boiling of the material in the bath, the shives, motes and, or, leaf are softened and put in such condition that they will be removed either mechanically as the material passes through the bath, or will be put in such condition that they will take the dye and be dyed a color the same as that of the other material, and in this way will be "removed" for the purposes of this invention, it being understood that a dyeing of the specks so that they cannot be detected by the eye is a "removal" in the sense in which that word is used in this case.

The materials used in the alkaline-oxidizing agent and the dye stuff must be selected so that they will not have mutual interfering action upon each other. It is found that the agent and such dye stuffs as are above mentioned do not have any mutual interfering action upon each other, but it is understood that the dye stuffs and other materials given are merely examples, and we are not limited to any given combination of dye stuffs and alkaline-oxidizing agent.

Having described our invention, what we claim as new and desire to secure by Letters Patent is:

1. The process of dyeing cotton material containing motes, shives and, or, leaf which consists in subjecting the same to an alkaline oxidizing bath adapted to soften the motes, shives and, or, leaf and to chemically attack the same, the bath containing also a direct or vegetable dye stuff of a composition substantially operatively unaffected by the other ingredients of said bath.

2. The process of dyeing cotton material containing motes, shives and, or, leaf, which consists in subjecting said material to an

- alkaline-oxidizing bath adapted to remove said motes, shives or leaf and subjecting said material to a dye-stuff operatively unaffected by said bath while it is in the said bath. 5
3. The process of dyeing uncombed cotton material containing motes, shives and, or, leaf, which consists in subjecting said material to an alkaline-oxidizing treatment in the presence of a dye operatively unaffected by said treatment. 10
4. The process of dyeing cotton material containing motes, shives and, or, leaf which consists in treating said material in an alkaline-oxidizing bath adapted to soften or loosen the motes, shives and, or, leaf and adding to said bath, while said material is therein, a dye stuff operatively unaffected by said bath. 15
- 20 5. The process of dyeing cotton material containing motes, shives and, or, leaf which consists in subjecting the same to an oxidizing bath including an alkaline substance adapted to soften the motes, shives or leaf and a substance adapted to chemically attack said motes, shives and, or, leaf, the bath containing also a dye-stuff of a composition substantially operatively unaffected by such mixture.
- 30 6. The process of dyeing cotton containing foreign matter which consists in subjecting said cotton to an alkaline-oxidizing bath containing a dye-stuff adapted to give the desired shade and operatively unaffected by said bath. 35
7. The process of dyeing cotton material containing specks of foreign matter which consists in boiling said material in the presence of an alkaline-oxidizing agent and a dyestuff substantially operatively unaffected by said agent. 40
- 45 8. The process of dyeing cotton material containing specks of foreign matter, which consists in subjecting said material to an alkaline-oxidizing bath to which a dye-stuff, substantially operatively unaffected by said bath, has been added and producing a continuous movement of the material in said bath to insure an even action of the bath upon said material. 50
- 55 9. The process of dyeing cotton material containing specks of foreign matter, which consists in boiling said material in an alkaline-oxidizing bath of strong alkalinity to which has been added a dye-stuff operatively unaffected by said bath. 60
- 60 10. The process of dyeing cotton material containing specks of foreign matter which consists in boiling said material in an alkaline-oxidizing bath and again in said bath with a dyestuff added thereto which is operatively unaffected by said bath. 65
11. The process of dyeing cotton material containing specks of foreign matter which consists in placing said material in a bath of water, adding ingredients to said bath to render it alkaline-oxidizing, bringing said bath to a boiling temperature, allowing said bath to partially cool, adding to said bath a dye-stuff operatively unaffected thereby, 70 gradually bringing said bath again to, and holding it at, a boiling temperature, allowing said bath to again partially cool, and maintaining it at the lesser temperature until the material is dyed. 75
12. The process of dyeing cotton material containing specks of foreign matter which consists in placing said material in a bath of water, adding ingredients to said bath to render it alkaline-oxidizing, bringing said bath to a boiling temperature, allowing said bath to partially cool to approximately 110° F., adding to said bath a dyestuff operatively unaffected thereby, gradually bringing said bath again to, and holding it at, a boiling 80 temperature for approximately fifteen to thirty minutes, allowing said bath to cool to approximately 190° F. and maintaining it at approximately that temperature until the material is dyed. 85
- 90 13. The process of dyeing cotton material containing specks of foreign matter which consists in boiling said material in an alkaline-oxidizing bath of marked alkalinity, adding to said bath a dyestuff operatively unaffected thereby and again boiling said material in said bath. 95
14. The process of dyeing cotton material containing specks of foreign matter which consists in subjecting said material to the action of a bath containing in solution a mixture of peroxid of sodium and an alkaline salt, adding to said bath a dyestuff operatively unaffected by said bath and boiling said material in the resulting bath. 100
- 105 15. The process of dyeing cotton material containing specks of foreign matter which consists in subjecting said material to the action of a bath containing in solution an amount equal to approximately 3% in weight of the material of approximately one-half peroxid of sodium and one-half an alkaline salt, adding to said bath a dyestuff operatively unaffected thereby and boiling said material in the resulting bath. 110
- 115 16. The process of dyeing cotton material containing specks of foreign matter, which consists in subjecting said material to a bath containing approximately equal amounts of peroxid of sodium and an alkaline sodium salt and adding to said bath a dye-stuff operatively unaffected thereby. 120
- In testimony whereof, we have signed our names to this specification.
- IRWIN J. SMITH.  
HARRY B. SMITH.